

# UNITED STATES PATENT OFFICE.

GEORGES HEBERLEIN, OF WATTWIL, SWITZERLAND.

## PROCESS FOR PRODUCING WOOLLIKE EFFECTS ON COTTON FABRICS.

1,141,872.

Specification of Letters Patent.

Patented June 1, 1915.

No Drawing.

Application filed May 28, 1914. Serial No. 841,594.

*To all whom it may concern:*

Be it known that I, GEORGES HEBERLEIN, a citizen of the Swiss Republic, and resident of Wattwil, Canton of St. Gall, Switzerland, have invented a New Process for Producing Woollike Effects on Cotton Fabrics, of which the following is a full, clear, and exact specification.

As observed by Mercer in 1844 and by others later, if concentrated sulfuric acid be caused to act on cotton, the cotton assumes a transparent parchment-like appearance. According to Mercer this effect is to be obtained with sulfuric acid of from 49.5° to 15 53.5° Bé., whereby the cellulose properties are altered. Blondell (*Bull. Rouen*, vol. 10, 1882, pages 438, 471-472) has however observed that sulfuric acid of 45° to 50° Bé. imparts to cellulose the property of being 20 capable of being readily dyed with methylene blue but imparts to it a parchment-like effect only when the concentration of the acid is from 53° to 55° Bé. (*Bull. Rouen*, vol. 10, 1882, page 471). As a matter of fact 25 sulfuric acid having a concentration of 51° Bé. and above, has an action on cellulose which is entirely different from the action thereon of acid whose concentration is below 51° Bé. Although more highly concentrated acid imparts to cotton after a few seconds' action a transparent parchment-like appearance, an acid of 50° Bé. for instance, even after acting for say, 15 minutes, will not cause a like alteration of the cellulose, 30 which however, in contradistinction to the effect of a slightly stronger acid, will not be weakened by even longer action.

The present invention is based on the observation that the action of sulfuric acid of 40 a concentration of less than 51° Bé. is much more intensive and imparts to cotton entirely new properties, if the cotton has previously been mercerized and thereby rendered more capable of being acted upon by the acid. If cotton fabric which has been mercerized and also preferably bleached, be subjected to the action of sulfuric acid of from 45 49° to 51° Bé. (the best action is obtained between 49.5° and 50.5° Bé.) the mercerizing 50 luster disappears and instead of the transparency obtained with the higher concentration the fabric assumes a fine, light, crape-like nature, whereby it appears fuller, more wool-like, softer, and is generally improved and it has imparted to it somewhat 55 the character of fine woolen stuff, the effect

being entirely new and hitherto unknown in cotton fabrics.

The invention can be employed for treating smooth, patterned, or embroidered, fabrics and patterned effect can be produced on plain cotton fabrics by printing on the mercerized fabrics with sulfuric acid of say 50° Bé. and washing out after printing. The fabric can also be printed on with a suitable 60 reserve (for instance, gum thickening) and then the fabric be dipped into sulfuric acid of the aforesaid concentration and washed out. In these cases, the places where the acid has acted, the fabric shows the aforesaid alteration, while the places which have 65 in the one case not been printed on by the acid and in the other case have been printed on by the reserve, preserve the appearance of the unchanged, mercerized cotton. In 70 this way it is possible to obtain patterns in which the lustrous, mercerized cotton is 75 prominently distinct from the dead, smooth wool-like parts treated with acids, as aforesaid.

The time during which the action of the sulfuric acid takes place depends upon the nature of the fabric to be dealt with. The alteration of the same may in some cases take place in a few minutes; but in others 80 it may require several minutes. A longer duration of the action than is necessary for the obtainment of the effect for instance 85 15 minutes, or more, has as a rule no injurious action.

In using sulfuric acid of from 50.5° to 51° Bé., which is capable of causing after an action of a few seconds' duration a transparent parchment-like effect on previously mercerized goods, the reaction in accordance with 90 the present invention takes a longer time, say, a few minutes.

What I claim is:

1. The described process for producing wool-like effects on cotton fabrics, consisting of taking mercerized fabrics and subjecting them for some minutes to the action of sulfuric acid of a concentration of from 49° to 51° Bé. and then washing out the acid. 100

2. The described process for the production of wool-like pattern effects on cotton fabrics consisting of subjecting for some minutes to the action of sulfuric acid of from 49° to 51° Bé. the places of mercerized cotton fabrics where pattern effects are to be 105 produced and then washing out the acid. 110

3. The described process for the produc-

tion of wool-like pattern effects on cotton fabrics consisting of printing the required pattern on mercerized cotton fabrics with sulfuric acid from 49° to 51° Bé. and finally 5 washing out the acid after some minutes.

In witness whereof I have hereunto signed

my name this 16 day of May 1914, in the presence of two subscribing witnesses.

GEORGES HEBERLEIN.

Witnesses:

E. T. HÖRLER,

C. UTENBER.